



US011920246B2

(12) **United States Patent**  
**Chen et al.**

(10) **Patent No.:** **US 11,920,246 B2**  
(45) **Date of Patent:** **Mar. 5, 2024**

(54) **SEAWATER ELECTROLYSIS ENABLES  
Mg(OH)<sub>2</sub> PRODUCTION AND CO<sub>2</sub>  
MINERALIZATION**

(71) Applicant: **The Regents of the University of  
California**, Oakland, CA (US)

(72) Inventors: **Xin Chen**, Los Angeles, CA (US);  
**Erika Callagon La Plante**, Los  
Angeles, CA (US); **Gaurav Sant**, Los  
Angeles, CA (US); **David Jassby**, Los  
Angeles, CA (US); **Dante Adam  
Simonetti**, Los Angeles, CA (US);  
**Thomas Traynor**, Los Angeles, CA  
(US)

(73) Assignee: **The Regents of the University of  
California**, Oakland, CA (US)

(\*) Notice: Subject to any disclaimer, the term of this  
patent is extended or adjusted under 35  
U.S.C. 154(b) by 0 days.

(21) Appl. No.: **17/968,596**

(22) Filed: **Oct. 18, 2022**

(65) **Prior Publication Data**

US 2023/0124711 A1 Apr. 20, 2023

**Related U.S. Application Data**

(60) Provisional application No. 63/256,888, filed on Oct.  
18, 2021.

(51) **Int. Cl.**  
**C25B 1/20** (2006.01)  
**C25B 9/19** (2021.01)  
(Continued)

(52) **U.S. Cl.**  
CPC ..... **C25B 1/20** (2013.01); **C25B 9/19**  
(2021.01); **C25B 9/30** (2021.01); **C25B 11/03**  
(2013.01);  
(Continued)

(58) **Field of Classification Search**  
CPC ..... C02F 1/4602  
See application file for complete search history.

(56) **References Cited**

**U.S. PATENT DOCUMENTS**

2,794,776 A \* 6/1957 Briggs ..... C02F 1/4618  
204/542  
3,655,537 A 4/1972 Russell et al.  
(Continued)

**FOREIGN PATENT DOCUMENTS**

CN 1137575 A 12/1996  
CN 101835727 B 8/2013  
(Continued)

**OTHER PUBLICATIONS**

“Mineral Makeup of Seawater”, available online at <https://web.stanford.edu/group/Urchin/mineral.html>, accessed on Feb. 21, 2023  
(Year: 2023).\*

(Continued)

*Primary Examiner* — Harry D Wilkins, III

(74) *Attorney, Agent, or Firm* — Foley Hoag LLP; David  
P. Halstead; Alexander J. Chatterley

(57) **ABSTRACT**

A method for producing one or more hydroxide solids includes providing a catholyte comprising an electrolyte solution; contacting the catholyte with an electroactive mesh cathode to electrolytically generate hydroxide ions, thereby precipitating the one or more hydroxide solid(s); and removing the one or more hydroxide solids from the surface of the mesh where they may deposit.

**30 Claims, 6 Drawing Sheets**



|      |                                            |                                                                                         |    |                            |                   |
|------|--------------------------------------------|-----------------------------------------------------------------------------------------|----|----------------------------|-------------------|
| (51) | <b>Int. Cl.</b>                            |                                                                                         | CN | 112981428 A                | 6/2021            |
|      | <i>C25B 9/30</i>                           | (2021.01)                                                                               | DE | 4326757 A1                 | 2/1994            |
|      | <i>C25B 11/03</i>                          | (2021.01)                                                                               | EP | 3673972 A1                 | 7/2020            |
|      | <i>C25B 11/046</i>                         | (2021.01)                                                                               | GB | 823531 A * 11/1959         | ..... C02F 1/4602 |
|      | <i>C25B 13/08</i>                          | (2006.01)                                                                               | IE | 922650 A1                  | 3/1994            |
|      | <i>C25B 15/08</i>                          | (2006.01)                                                                               | WO | WO 87/01108 A1 * 2/1987    | ..... C02F 1/4602 |
| (52) | <b>U.S. Cl.</b>                            |                                                                                         | WO | WO 2009/039445 A2          | 3/2009            |
|      | CPC .....                                  | <b>C25B 11/046</b> (2021.01); <b>C25B 13/08</b> (2013.01); <b>C25B 15/08I</b> (2021.01) | WO | WO 2012/095659 A1 * 7/2012 | ..... C02F 1/4602 |
| (56) | <b>References Cited</b>                    |                                                                                         | WO | WO-2016/028023 A1          | 2/2016            |
|      | U.S. PATENT DOCUMENTS                      |                                                                                         | WO | WO-2018/218294 A1          | 12/2018           |
|      | 3,725,259 A 4/1973 Depree                  |                                                                                         | WO | WO-2021/097518 A1          | 5/2021            |
|      | 3,790,464 A * 2/1974 Greaves .....         | C25B 9/30                                                                               | WO | WO 2021/117934 A1 * 6/2021 | ..... C25B 15/00  |
|      |                                            | 204/268                                                                                 | WO | WO-2023/278423 A1          | 1/2023            |
|      | 4,069,117 A 1/1978 Cooper                  |                                                                                         | WO | WO-2023/069777 A1          | 4/2023            |
|      | 4,671,863 A * 6/1987 Tejeda .....          | C02F 1/4604                                                                             | WO | WO-2023/069947 A2          | 4/2023            |
|      |                                            | 204/266                                                                                 |    |                            |                   |
|      | 5,043,017 A 8/1991 Passaretti              |                                                                                         |    |                            |                   |
|      | 5,362,460 A 11/1994 Laird                  |                                                                                         |    |                            |                   |
|      | 5,543,034 A * 8/1996 Hilbertz .....        | A01K 61/50                                                                              |    |                            |                   |
|      |                                            | 204/DIG. 6                                                                              |    |                            |                   |
|      | 6,228,161 B1 5/2001 Drummond               |                                                                                         |    |                            |                   |
|      | 11,040,898 B2 6/2021 Sant et al.           |                                                                                         |    |                            |                   |
|      | 11,413,578 B2 8/2022 Sant et al.           |                                                                                         |    |                            |                   |
|      | 2002/0179435 A1 * 12/2002 Maddan .....     | C25B 1/20                                                                               |    |                            |                   |
|      |                                            | 204/263                                                                                 |    |                            |                   |
|      | 2003/0213937 A1 11/2003 Yaniv              |                                                                                         |    |                            |                   |
|      | 2004/0253417 A1 12/2004 Sekoguchi et al.   |                                                                                         |    |                            |                   |
|      | 2005/0180910 A1 8/2005 Park                |                                                                                         |    |                            |                   |
|      | 2005/0242032 A1 11/2005 Sugito et al.      |                                                                                         |    |                            |                   |
|      | 2009/0001020 A1 1/2009 Constantz           |                                                                                         |    |                            |                   |
|      | 2009/0013742 A1 1/2009 Zhang               |                                                                                         |    |                            |                   |
|      | 2009/0056707 A1 3/2009 Foody               |                                                                                         |    |                            |                   |
|      | 2009/0214408 A1 8/2009 Blake et al.        |                                                                                         |    |                            |                   |
|      | 2010/0034724 A1 2/2010 Keith et al.        |                                                                                         |    |                            |                   |
|      | 2010/0150803 A1 6/2010 Lin                 |                                                                                         |    |                            |                   |
|      | 2010/0260653 A1 10/2010 Jones              |                                                                                         |    |                            |                   |
|      | 2011/0195017 A1 8/2011 Martinez Martinez   |                                                                                         |    |                            |                   |
|      | 2012/0090433 A1 4/2012 Butler              |                                                                                         |    |                            |                   |
|      | 2012/0156126 A1 6/2012 Blunn et al.        |                                                                                         |    |                            |                   |
|      | 2012/0186492 A1 7/2012 Gane et al.         |                                                                                         |    |                            |                   |
|      | 2013/0034489 A1 2/2013 Gilliam et al.      |                                                                                         |    |                            |                   |
|      | 2013/0313199 A1 11/2013 Marcin et al.      |                                                                                         |    |                            |                   |
|      | 2015/0307400 A1 10/2015 Devenney           |                                                                                         |    |                            |                   |
|      | 2016/0090656 A1 * 3/2016 Livni .....       | C25B 15/00                                                                              |    |                            |                   |
|      |                                            | 205/350                                                                                 |    |                            |                   |
|      | 2016/0194208 A1 7/2016 Lake et al.         |                                                                                         |    |                            |                   |
|      | 2016/0362800 A1 12/2016 Ren et al.         |                                                                                         |    |                            |                   |
|      | 2017/0191173 A1 7/2017 Han et al.          |                                                                                         |    |                            |                   |
|      | 2017/0291832 A1 * 10/2017 Salama .....     | B06B 1/0618                                                                             |    |                            |                   |
|      | 2019/0329176 A1 10/2019 Lu et al.          |                                                                                         |    |                            |                   |
|      | 2019/0367390 A1 12/2019 Sant et al.        |                                                                                         |    |                            |                   |
|      | 2020/0122090 A1 4/2020 Kitaura et al.      |                                                                                         |    |                            |                   |
|      | 2020/0385280 A1 12/2020 Dai et al.         |                                                                                         |    |                            |                   |
|      | 2021/0123146 A1 4/2021 Berlinguette et al. |                                                                                         |    |                            |                   |
|      | 2021/0188671 A1 6/2021 Sant et al.         |                                                                                         |    |                            |                   |
|      | 2021/0308623 A1 10/2021 Sorimachi          |                                                                                         |    |                            |                   |
|      | 2022/0040639 A1 2/2022 Sant et al.         |                                                                                         |    |                            |                   |
|      | 2022/0176311 A1 6/2022 Omosebi et al.      |                                                                                         |    |                            |                   |
|      | 2022/0267159 A1 8/2022 Shi et al.          |                                                                                         |    |                            |                   |
|      | 2023/0019754 A1 1/2023 Sant et al.         |                                                                                         |    |                            |                   |
|      | 2023/0058065 A1 2/2023 Sant et al.         |                                                                                         |    |                            |                   |
|      | 2023/0124711 A1 4/2023 Chen et al.         |                                                                                         |    |                            |                   |
|      | 2023/0125242 A1 4/2023 Sant et al.         |                                                                                         |    |                            |                   |

## FOREIGN PATENT DOCUMENTS

|    |             |         |
|----|-------------|---------|
| CN | 107201443 A | 9/2017  |
| CN | 107268027 A | 10/2017 |

## OTHER PUBLICATIONS

- Van Treeck et al., Artificial Reefs Created by Electrolysis and Coral Transplantation: An Approach Ensuring the Compatibility of Environmental Protection and Diving Tourism, Estuarine, Coastal and Shelf Science, vol. 49, Supplement 1, Aug. 1999, pp. 75-81 (Year: 1999).\*
- Carré et al, Electrochemical calcerous deposition in seawater. A review, Environmental Chemistry Letters, vol. 18, Apr. 2020, pp. 1193-1208 (Year: 2020).\*
- Karoui et al, Electrochemical scaling of stainless steel in artificial seawater: Role of experimental conditions on CaCO<sub>3</sub> and Mg(OH)<sub>2</sub> formation, Desalination, vol. 311, Feb. 2013, pp. 234-240 (Year: 2013).\*
- Bisericic et al., "Ultrasound and shacking-assisted water-leaching of anions and cations from fly ash" J. Serb. Chem. Soc. 81 (7) 813-827 (2016).
- International Search Report and Written Opinion dated Mar. 25, 2021, from application No. PCT/US2020/037629, 10 pages.
- International Search Report and Written Opinion for Application No. PCT/US2022/0478585 dated Mar. 28, 2023.
- International Search Report and Written Opinion for International Application No. PCT/US22/35289 dated Oct. 27, 2022.
- Jun-Hwan Bang, et al., "CO<sub>2</sub> Mineralization Using Brine Discharged from a Seawater Desalination Plant," Abstract, Minerals, Vo.7, No. 207, Oct. 30, 2017, pp. 1-12.
- Socolow et al. "Direct air capture of CO<sub>2</sub> with chemicals: a technology assessment for the APS Panel on Public Affairs", American Physical Society, (2011).
- Translation of CN 101835727 B.
- Translation of CN-107201443.
- Translation of CN-113005471.
- Translation of CN-207699684.
- U.S. Office Action for U.S. Appl. No. 16/431,300 dated Jan. 25, 2021.
- Extended European Search Report for EP Application No. 20867650.2 dated Sep. 12, 2023.
- International Search Report and Written Opinion for Application No. PCT/US2022/078300 dated May 23, 2023.
- Khajouei G. et al. "Produced water softening using high-pH catholyte from brine electrolysis: reducing chemical transportation and environmental footprints." Journal of Water Process Engineering, vol. 40, 2021, Article 101911, pp. 1-9.
- La Plante E.C. et al. "Saline Water-Based Mineralization Pathway for Gigatonne-Scale CO<sub>2</sub> Management." ACS Sustainable Chemistry & Engineering, vol. 9, Issue 3, 2021, pp. 1073-1089.
- Partial Supplementary European Search Report for Application No. EP dated Jun. 9, 2023.
- Zhang Y. et al. "The use and optimization of stainless steel mesh cathodes in microbial electrolysis cells." International Journal of Hydrogen Energy, vol. 35, Issue 21, 2010, pp. 12020-12028.

\* cited by examiner



FIG. 1A



FIG. 1B



FIG. 2



FIG. 3A



FIG. 3B



FIG. 3C

## 1

**SEAWATER ELECTROLYSIS ENABLES  
Mg(OH)<sub>2</sub> PRODUCTION AND CO<sub>2</sub>  
MINERALIZATION**

**CROSS-REFERENCE TO RELATED  
APPLICATIONS**

This application claims the benefit of priority to U.S. Provisional Application No. 63/256,888, filed on Oct. 18, 2021, the contents of which are hereby incorporated by reference in their entirety.

**STATEMENT OF GOVERNMENT SUPPORT**

This invention was made with government support under DE-FE0031705 awarded by the Department of Energy. The government has certain rights in the invention.

**BACKGROUND OF THE INVENTION**

Ocean carbon storage is a pathway for reducing atmospheric carbon concentrations. The oceans represent a vast reservoir of about 38,000 gigatonnes of carbon<sup>1</sup>, stored in a dissolved form as H<sub>2</sub>CO<sub>3</sub>, CO<sub>3</sub><sup>2-</sup>, and CO<sub>3</sub><sup>2-</sup> species. Carbon capture from oceans via the formation of divalent metal carbonate solids from ocean water has the potential to decrease its carbon storage capacity due to a pH reduction from this process. But an increase in the pH of ocean water may increase this storage capacity in accordance with Henry's law (see, e.g., FIG. 1A, showing a plot of seawater CO<sub>2</sub> uptake with respect to pH). Accordingly, the addition of alkaline materials, such as metal hydroxides, to ocean water has the potential to increase its pH, thereby restoring its carbon storage capacity.

Brucite (Mg(OH)<sub>2</sub>) for industrial uses can be obtained either naturally, through the hydration of MgO produced from calcining magnesium carbonate, or by precipitation from seawater by the provision of alkalinity. Ocean water contains a high amount of Mg<sup>2+</sup> ions, particularly in the form of chloride and sulfate salts. Thus, ocean water can be a source for brucite production. There is a need for efficient methods of forming brucite from ocean water. There is further a need for methods of increasing pH of ocean water, particularly as a part of carbon capture methods.

**SUMMARY**

The present disclosure relates to methods for producing hydroxide solids, particularly Mg(OH)<sub>2</sub> solids. In some embodiments, the present disclosure provides a method for producing one or more hydroxide solids, the method comprising:

providing a catholyte comprising an electrolyte solution; p contacting the catholyte with an electroactive mesh cathode to electrolytically generate hydroxide ions, thereby precipitating the one or more hydroxide solids.

In some embodiments, the electrolyte solution comprises divalent metal cations. In certain embodiments, the electrolyte solution comprises Mg<sup>2+</sup>, Ca<sup>2+</sup>, or both Mg<sup>2+</sup> and Ca<sup>2+</sup> ions. In particularly preferred embodiments, the divalent cations comprise Mg<sup>2+</sup> ions.

In certain embodiments, wherein the electrolyte solution comprises a brine or sea water. Preferably, the electrolyte solution comprises sea water.

In certain embodiments, the brine or sea water comprises NaCl in the brine or sea water in a concentration about 1,000 ppm or more, about 2,000 ppm or more, about 3,000 ppm or

## 2

more, about 4,000 ppm or more, about 5,000 ppm or more, about 6,000 ppm or more, about 7,000 ppm or more, about 8,000 ppm or more, about 9,000 ppm or more, about 10,000 ppm or more, about 15,000 ppm or more, about 20,000 ppm or more, about 25,000 ppm or more, or about 30,000 ppm or more, about 35,000 ppm or more, about 40,000 ppm or more, about 45,000 ppm or more, about 50,000 ppm or more, about 55,000 ppm or more, or about 60,000 ppm or more. Preferably, the NaCl concentration is about 35,000 or more.

In certain embodiments, the electrolyte solution has a Ca-equivalent or Mg-equivalent concentration of about 2 ppm or more, about 10 ppm or more, about 50 ppm or more, about 100 ppm or more, about 200 ppm or more, about 300 ppm or more, about 400 ppm or more, about 500 ppm or more, about 600 ppm or more, about 700 ppm or more, about 800 ppm or more, about 900 ppm or more, about 1000 ppm or more, about 11 ppm or more, about 1200 ppm or more, about 1300 ppm or more, about 1400 ppm or more, or about 1500 ppm or more. Preferably, the electrolyte solution has an 15 Mg-equivalent concentration of about 1000 ppm or more.

In some embodiments, the one or more hydroxide solids comprises Mg(OH)<sub>2</sub>, Ca(OH)<sub>2</sub>, or both Mg(OH)<sub>2</sub> and Ca(OH)<sub>2</sub>. Preferably, the one or more hydroxide solids comprise Mg(OH)<sub>2</sub>.

In some embodiments, the electroactive mesh cathode comprises a rotating disc cathode. In particular embodiments, the rotating disc cathode has an electroactive mesh disposed thereon.

In some embodiments, the method further comprises removing the one or more hydroxide solids from the surface of the mesh. In particular embodiments, the removing the one or more hydroxide solids from the surface of the mesh comprises scraping the surface of the mesh.

In some embodiments where the cathode is a rotating disc cathode, removing the one or more hydroxide solids from the surface of the mesh comprises rotating the rotating disc cathode past a scraper.

In certain embodiments, the electroactive mesh cathode comprises a metallic composition, non-metallic composition, or hybrid metallic and non-metallic composition.

40 In some embodiments, the electroactive mesh cathode comprises stainless steel, titanium oxide, carbon nanotubes, one or more polymers, graphite, or combinations thereof. Preferably, the mesh cathode comprises stainless steel.

In some embodiments, the electroactive mesh comprises 45 pores having a diameter in the range of about 0.1 μm to about 10000 μm.

In some embodiments, the method comprises forming alkalized effluents having a pH greater than 9, or in other embodiments, greater than 10.

In some embodiments, the anolyte comprises an acid. In certain embodiments, the acid has a pH of less than about 6.

In some embodiments, the method further comprises providing a barrier to separate the catholyte and the anolyte. In some embodiments, the barrier comprises a polymer, such as cellulose, polyvinyl chloride, organic rubber, polyolefin, polyethylene, polypropylene, or any combination thereof.

In other embodiments, the method further comprises cycling the anolyte to a neutralization pool. The neutralization pool may comprise mafic materials, ultramafic materials, calcium-rich fly ash, slag, or any combination thereof.

60 In some embodiments, the electrolytically generating of hydroxide ions is conducted at a current density of greater than 50 μA/cm<sup>2</sup>.

**BRIEF DESCRIPTION OF THE DRAWINGS**

65 FIG. 1A is a plot of seawater CO<sub>2</sub> uptake capacity with respect to pH.

FIG. 1B is a plot of the enhancement of seawater's CO<sub>2</sub> uptake capacity by Mg(OH)<sub>2</sub> dissolution.

FIG. 2 is a schematic illustration of a brucite mineralization reactor, in accordance with various embodiments.

FIG. 3A is a plot of brucite production and removal rate per 1 L of seawater as a function of current densities.

FIG. 3B is a scanning electron microscopy (SEM) image of brucite precipitates formed on a cathode.

FIG. 3C is an x-ray diffraction (XRD) pattern of brucite precipitates formed on a cathode.

## DETAILED DESCRIPTION

The process according to the present disclosure is based on electrochemically enhanced electrolysis reactions to form brucite (Mg(OH)<sub>2</sub>) precipitates in order to increase ocean alkalinity and promote atmospheric carbon dioxide dissolution. Such processes include, but are not limited to, those disclosed in International Application No. PCT/US22/35289 filed on Jun. 28, 2022, International Application PCT/US20/37629 filed on Jun. 12, 2020, and U.S. application Ser. No. 17/722,036 filed on Apr. 15, 2022, the entireties of which are hereby incorporated by reference herein.

As shown in FIG. 1A, increasing the pH of seawater increases its carbon storage capacity according to the equilibrium constants describing the speciation of H<sub>2</sub>CO<sub>3</sub>, HCO<sub>3</sub><sup>-</sup>, and CO<sub>3</sub><sup>2-</sup> ions and Henry's Law. In particular, the dissolution of alkaline (e.g., calcium- and magnesium-rich) solids in the ocean surface could advantageously increase its pH, allowing additional CO<sub>2</sub> uptake. The CO<sub>2</sub> uptake (quantified as a mass of CO<sub>2</sub> incorporated into solid products or as dissolved ions per mass of initial solid or liquid material) describes the material's efficiency in sequestering gaseous CO<sub>2</sub> in stable solids or dissolved ions. Enhancing CO<sub>2</sub> uptake allows impactful removal of gaseous CO<sub>2</sub> resulting from anthropogenic sources.

As shown in FIG. 1B, brucite (Mg(OH)<sub>2</sub>) may be added in seawater to equilibrium which results in a pH of 9.1, equivalent to about a threefold increase in the total dissolved CO<sub>2</sub>, compared to that at pH of 8.2, which is the typical pH of seawater. Brucite for industrial uses can be obtained either naturally, e.g., through the hydration of MgO produced from calcining magnesium carbonate, or by precipitation from seawater by the provision of alkalinity. FIG. 1B illustrates CO<sub>2</sub> uptake capacity enhanced by brucite dissolution. Every mole of dissolved brucite can promote about 1.6 moles of atmospheric CO<sub>2</sub> absorption.

In the present disclosure, metal hydroxide solids, such as brucite, may be produced by an electrochemical process that uses seawater, which contains ~55 mmol Mg/L, or using other Mg-rich brines as feeds. In some embodiments, a membrane-less reactor may be used to produce brucite precipitates. Advantages of such a membrane-less reactor may include lower energy requirements, reduced maintenance and operating costs, and reduced manufacturing expense at increasing scales.

In some embodiments, a method according to the present disclosure comprises: providing a catholyte comprising an electrolyte solution; contacting the catholyte with an electroactive mesh cathode to electrolytically generate hydroxide ions, thereby precipitating the one or more hydroxide solids.

In some embodiments, the method further comprises removing the one or more hydroxide solids from the surface of the mesh where they may deposit.

A CO<sub>2</sub> mineralization process can be achieved by alkalinizing a circumneutral Ca- and Mg-containing solution (e.g.,

seawater, alkaline metal-rich groundwater, industrial wastewater, or desalination brine). In some embodiments, the method uses a single-compartment continuous stirred-tank reactor (CSTR). Operational parameters such as voltage, current density, and hydraulic retention time ("HRT")) are chosen to minimize the hydroxylation energy intensity of the design.

Turning to FIG. 2, a membrane-less reactor useful for practicing certain embodiments of the present invention is shown. A membrane-less electrolysis reactor 200 was conceptualized to electrochemically precipitate hydroxide solids from a catholyte. In some embodiments, a hydroxide-forming process can advantageously be achieved by alkalinizing a circumneutral Ca- and Mg-containing solution, such as seawater, alkaline metal-rich groundwater, industrial wastewater, or desalination brine. We evaluated the feasibility of the conceptualized multi-compartment reactor, by using a single-compartment continuous stirred-tank reactor (CSTR). Operational parameters (e.g., voltage, current density, and hydraulic retention time ("HRT")) may also be selected to demonstrate the carbonation energy intensity of the design.

Referring still to FIG. 2, reactor 200 includes a reservoir 405 containing a catholyte, such as seawater, alkaline metal-rich groundwater, industrial wastewater, desalination brine. The reactor further includes an anolyte inlet 203 and outlet 211. Electrode assembly 206 is in fluid contact with the aqueous sequestration solution reservoir 205 and comprises rotating disk cathodes 207 and anodes 209 separated by a barrier layer 208. The rotating disc cathodes 207 (e.g. 316L stainless steel mesh) may be rotated around shaft 202 to pass a scraper 210 for product removal and collection. The reactor may further comprise a neutralization pool 212. O<sub>2</sub> may be produced at the anode 209, and may be released at an O<sub>2</sub> outlet 213. H<sub>2</sub> may be produced at the rotating disk cathode 207, and may be released at an H<sub>2</sub> outlet 214.

In embodiments comprising rotating disc cathodes, inducing the precipitation of the carbonate solid includes rotating a cylinder consisting of the electroactive mesh in the solution, while applying suction to draw the solution onto the outer surface of the mesh.

The electrolytes may be separated with a porous barrier for the following reasons: (1) minimized neutralization reactions between anolytes and catholytes allows stable cathode pH for effective mineralization; (2) separated electrolytes promote higher energy efficiency of the reactor; and (3) the gas streams (H<sub>2</sub> and O<sub>2</sub>) may need to be divided and collected separately.

Referring still to FIG. 2, an online pH-monitoring system 50 may be used, for example, to control the applied electric current to attain a constant catholyte pH or greater than 9. The anolyte can in some embodiments provide

In some embodiments, the reactor includes a catholyte and an anolyte. The catholyte may be an electrolyte solution 55 configured to flow around or through a cathode. The anolyte may be an electrolyte configured to flow around or through an anode. The catholyte may comprise an electrolyte solution.

In some embodiments, the electrolyte solution comprises 60 divalent metal cations, such as Mg<sup>2+</sup>, Ca<sup>2+</sup>, or both Mg<sup>2+</sup> and Ca<sup>2+</sup> ions. In particularly preferred embodiments, the electrolyte solution comprises Mg<sup>2+</sup> ions.

In some embodiments, the electrolyte solution comprises 65 seawater or a brine. Preferably, the electrolyte is seawater. In some embodiments, the electrolyte solution has a concentration of NaCl of about 1,000 ppm or more, about 2,000 ppm or more, about 3,000 ppm or more, about 4,000 ppm or

more, about 5,000 ppm or more, about 6,000 ppm or more, about 7,000 ppm or more, about 8,000 ppm or more, about 9,000 ppm or more, about 10,000 ppm or more, about 15,000 ppm or more, about 20,000 ppm or more, about 25,000 ppm or more, or about 30,000 ppm or more, about 35,000 ppm or more, about 40,000 ppm or more, about 45,000 ppm or more, about 50,000 ppm or more, about 55,000 ppm or more, or about 60,000 ppm or more, or greater, or any range or value there between. In preferred embodiments, the electrolyte solution has a NaCl concentration of about 35,000 ppm or more.

In some embodiments, the catholyte has a concentration of Ca-equivalent or Mg-equivalent of about 2 ppm or more, about 10 ppm or more, about 50 ppm or more, about 100 ppm or more, about 200 ppm or more, about 300 ppm or more, about 400 ppm or more, about 500 ppm or more, about 600 ppm or more, about 700 ppm or more, about 800 ppm or more, about 900 ppm or more, about 1000 ppm or more, about 11 ppm or more, about 1200 ppm or more, about 1300 ppm or more, about 1400 ppm or more, or about 1500 ppm or more. Preferably, the catholyte solution has an Mg-equivalent concentration of about 1000 ppm or more. Ca-equivalent and Mg-equivalent refer to salts of Ca and Mg in the electrolyte solution. Preferably, the salts are chloride salts or sulfate salts.

In some embodiments, the anolyte comprises an acid. In some embodiments, the anolyte has a pH of less than about 7, less than about 6, less than about 4, less than about 3, less than about 2, down to less than about 1. In particular embodiments, the anolyte has a pH of about 1 to about 6, about 1 to about 5, about 1 to about 4, about 1 to about 3, or about 1 to about 2.

In some embodiments, the one or more hydroxide solids comprise  $Mg(OH)_2$ ,  $Ca(OH)_2$ , or both  $Mg(OH)_2$  and  $Ca(OH)_2$ . In particularly preferred embodiments, the one or more hydroxide solids comprise  $Mg(OH)_2$  (also referred to herein as brucite).

In some embodiments, the cathode 207 comprises an electroactive mesh. In some embodiments, the electroactive mesh comprises a metallic or a non-metallic composition, or a combination of metallic and non-metallic compositions. In some embodiments, the electroactive mesh comprises, consists essentially of, or consists of a metallic mesh or carbon-based mesh. In some embodiments, the electroactive mesh comprises stainless steel, titanium oxide, carbon nanotubes, polymers, and/or graphite, or other hybrid compositions of these materials. Preferably, the electroactive mesh comprises stainless.

In some embodiments, the electroactive mesh comprises pores having a diameter in the range of about 0.01  $\mu m$  to about 10000  $\mu m$  (e.g., about 0.1, 0.2, 0.3, 0.4, 0.5, 0.6, 0.7, 0.8, 0.9, 1, 2, 3, 4, 5, 6, 7, 8, 9, 10, 20, 30, 40, 50, 60, 70, 80, 90, 100, 200, 300, 400, 500, 1000, 1500, 2000, 3000, 4000, 5000, 6000, 7000, 8000, 9000, or 10000  $\mu m$ , or any range there between).

In some embodiments, the cathodes 207 are (for example, 316L stainless steel mesh) coupled with OER-(oxygen evolution reactions) selective anodes (e.g.,  $MnO_2$ -coated Pt) to produce alkalinity and acidity.

In some embodiments, the method further comprises removing the one or more hydroxide solids from the surface of the mesh. In preferred embodiments, the one or more hydroxide solids are removed by a scraping process. The scraping process may use a metallic brush, blade, or high-pressure nozzles. In particular embodiments where the cathodes are rotating disc cathodes, the one or more hydroxide

solids from the surface of the mesh may be removed from the surface of the mesh by rotating the rotating disc cathode past a scraper,

In some embodiments, the reactor further comprises a barrier 208 to separate the anolyte from the catholyte. In some embodiments, the barrier comprises cellulose, polyvinyl chloride, organic rubber, polyolefin, polyethylene, polypropylene, any other suitable material, or combinations thereof. The barrier separates the catholyte and anolyte in order to: (1) minimize neutralization reactions between the anolyte and the catholyte, resulting in a stable cathode pH necessary for brucite production; (2) promote higher energy efficiency of the reactor; and (3) facilitate collection of gas streams ( $H_2$  and  $O_2$ ).

A pH-monitoring system may be used, for example, to control the applied electric current to attain a constant catholyte pH. For example, in some embodiments, the catholyte pH is maintained above 9, such as at about 9.5-9.6. The stainless steel cathodes may be covered by a hydrophobic mesh (e.g., polypropylene (PP) meshes) as hydroxide catalysts, thereby electrolytically generating hydroxide ions at the cathode. The catholyte may be seawater-flushed such that the  $Mg^{2+}$  ions react with the electrolytically produced  $OH^-$  ions to produce  $Mg(OH)_2$ . Operational parameters including current density and hydraulic retention time, and HRT may be optimized. Within a reasonable HRT (e.g., in seconds to minutes), the production of  $Mg(OH)_2$  is promoted at high current densities. In some embodiments, the current density is greater than 50  $\mu A/cm^2$ , greater than 100  $\mu A/cm^2$ , greater than 200  $\mu A/cm^2$ , greater than 300  $\mu A/cm^2$ , greater than 400  $\mu A/cm^2$ , or greater than 5000  $\mu A/cm^2$ , or at any range therebetween. In addition, high current densities may also yield alkalinized effluents (e.g., pH greater than about 9, or greater than about 10), can advantageously be used to improve  $CO_2$  capture capabilities of an anolyte source, such as seawater.

In some embodiments, PP-covered stainless steel cathodes may be rotated to pass a scraper (e.g., a metallic brush, blade, or high-pressure nozzles) to remove the hydroxides, thereby regenerating the cathode for subsequent hydroxide production as the discs rotate back into the liquid. In some embodiments, a nozzle sprayer may be used to force the detachment of the precipitated hydroxides.

In some embodiments, the anolyte is cycled to a neutralization pool 212 comprising calcium-rich fly ash, slag, or any combination thereof, and the produced acidity can thus be consumed to restore alkalinity. Ca-rich fly ashes and minerals advantageously may also be used to enrich the  $Ca^{2+}$  in anolyte.

As shown in FIGS. 3A-C,  $Mg(OH)_2$  according to certain embodiments of the present methods forms a scale at the cathode surface, permitting easy removal via a simple scraping process. FIG. 3A shows a plot of the brucite production and removal rates per L seawater as functions of the current densities. A higher current density yields a lower concentration of brucite formed and a higher removal rate. FIG. 3B shows a scanning electron microscopy (SEM) image of the brucite precipitates formed on the cathode mesh. The brucite formed is thick, brittle, and with defined cracks, which help promote easy removal. FIG. 3C shows an X-ray diffraction (XRD) plot of the precipitates formed. The XRD plot shows that brucite is formed as the same peaks are seen between the precipitates and brucite.

As used herein, the singular terms "a," "an," and "the" include plural referents unless the context clearly dictates

otherwise. Thus, for example, reference to an object can include multiple objects unless the context clearly dictates otherwise.

As used herein, the term “set” refers to a collection of one or more objects. Thus, for example, a set of objects can include a single object or multiple objects.

As used herein, the terms “substantially” and “about” are used to describe and account for small variations. When used in conjunction with an event or circumstance, the terms can refer to instances in which the event or circumstance occurs precisely as well as instances in which the event or circumstance occurs to a close approximation. For example, when used in conjunction with a numerical value, the terms can encompass a range of variation of less than or equal to  $\pm 10\%$  of that numerical value, such as less than or equal to  $\pm 5\%$ , less than or equal to  $\pm 4\%$ , less than or equal to  $\pm 3\%$ , less than or equal to  $\pm 2\%$ , less than or equal to  $\pm 1\%$ , less than or equal to  $\pm 0.5\%$ , less than or equal to  $\pm 0.1\%$ , or less than or equal to  $\pm 0.05\%$ .

As used herein, the term “size” refers to a characteristic dimension of an object. Thus, for example, a size of an object that is circular can refer to a diameter of the object. In the case of an object that is non-circular, a size of the non-circular object can refer to a diameter of a corresponding circular object, where the corresponding circular object exhibits or has a particular set of derivable or measurable characteristics that are substantially the same as those of the non-circular object. Alternatively, or in conjunction, a size of a non-circular object can refer to an average of various orthogonal dimensions of the object. Thus, for example, a size of an object that is an ellipse can refer to an average of a major axis and a minor axis of the object. When referring to a set of objects as having a particular size, it is contemplated that the objects can have a distribution of sizes around the particular size. Thus, as used herein, a size of a set of objects can refer to a typical size of a distribution of sizes, such as an average size, a median size, or a peak size.

Additionally, amounts, ratios, and other numerical values are sometimes presented herein in a range format. It is to be understood that such range format is used for convenience and brevity and should be understood flexibly to include numerical values explicitly specified as limits of a range, but also to include all individual numerical values or sub-ranges encompassed within that range as if each numerical value and sub-range is explicitly specified. For example, a ratio in the range of about 1 to about 200 should be understood to include the explicitly recited limits of about 1 and about 200, but also to include individual ratios such as about 2, about 3, and about 4, and sub-ranges such as about 10 to about 50, about 20 to about 100, and so forth.

While the disclosure has been described with reference to the specific embodiments thereof, it should be understood by those skilled in the art that various changes may be made and equivalents may be substituted without departing from the true spirit and scope of the disclosure as defined by the appended claims. In addition, many modifications may be made to adapt a particular situation, material, composition of matter, method, operation or operations, to the objective, spirit and scope of the disclosure. All such modifications are intended to be within the scope of the claims appended hereto. In particular, while certain methods may have been described with reference to particular operations performed in a particular order, it will be understood that these operations may be combined, sub-divided, or re-ordered to form an equivalent method without departing from the teachings

of the disclosure. Accordingly, unless specifically indicated herein, the order and grouping of the operations is not a limitation of the disclosure.

The embodiments, illustratively described herein may suitably be practiced in the absence of any element or elements, limitation or limitations, not specifically disclosed herein. Thus, for example, the terms “comprising,” “including,” “containing,” etc. shall be read expansively and without limitation. Additionally, the terms and expressions employed herein have been used as terms of description and not of limitation, and there is no intention in the use of such terms and expressions of excluding any equivalents of the features shown and described or portions thereof, but it is recognized that various modifications are possible within the scope of the claimed technology. Additionally, the phrase “consisting essentially of” will be understood to include those elements specifically recited and those additional elements that do not materially affect the basic and novel characteristics of the claimed technology. The phrase “consisting of” excludes any element not specified.

## REFERENCES

1. Renforth, P.; Henderson, G. Assessing Ocean Alkalinity for Carbon Sequestration. *Rev. Geophys.* 2017, 55 (3), 636-674. <https://doi.org/10.1002/2016RG000533>.
2. Kheshgi, H. S. Sequestering Atmospheric Carbon Dioxide by increasing Ocean Alkalinity. *Energy* 1995, 20 (9), 915-922. [https://doi.org/10.1016/0360-5442\(95\)00035-F](https://doi.org/10.1016/0360-5442(95)00035-F).

## INCORPORATION BY REFERENCE

All publications and patents mentioned herein are hereby incorporated by reference in their entirety as if each individual publication or patent was specifically and individually indicated to be incorporated by reference. In case of conflict, the present application, including any definitions herein, will control.

## EQUIVALENTS

While specific embodiments of the subject invention have been discussed, the above specification is illustrative and not restrictive. Many variations of the invention will become apparent to those skilled in the art upon review of this specification and the claims below. The full scope of the invention should be determined by reference to the claims, along with their full scope of equivalents, and the specification, along with such variations.

The invention claimed is:

1. A method for producing one or more hydroxide solids, the method comprising:  
providing:  
a basic catholyte solution comprising an electrolyte;  
an acidic anolyte solution; and  
a neutralization pool comprising an alkaline material;  
contacting the basic catholyte solution with an electroactive mesh cathode to electrolytically generate hydroxide ions, thereby precipitating the one or more hydroxide solids; and  
circulating the acidic anolyte solution through the neutralization pool, thereby forming a neutral anolyte solution.
2. The method of claim 1, wherein in the electrolyte comprises divalent metal cations.
3. The method of claim 2, wherein the divalent cations comprise  $Mg^{2+}$ ,  $Ca^{2+}$ , or both  $Mg^{2+}$  and  $Ca^{2+}$  ions.

4. The method of claim 3, wherein the divalent cations comprise Mg<sup>2+</sup> ions.

5. The method of claim 1, wherein the electrolyte comprises a brine or sea water.

6. The method of claim 5, wherein the electrolyte comprises sea water.

7. The method of claim 5, wherein the concentration of NaCl in the brine or sea water is about 1,000 ppm or more, about 2,000 ppm or more, about 3,000 ppm or more, about 4,000 ppm or more, about 5,000 ppm or more, about 6,000 ppm or more, about 7,000 ppm or more, about 8,000 ppm or more, about 9,000 ppm or more, about 10,000 ppm or more, about 15,000 ppm or more, about 20,000 ppm or more, about 25,000 ppm or more, or about 30,000 ppm or more, about 35,000 ppm or more, about 40,000 ppm or more, about 45,000 ppm or more, about 50,000 ppm or more, about 55,000 ppm or more, or about 60,000 ppm or more.

8. The method of claim 1, wherein the electrolyte has a Ca-equivalent or Mg-equivalent concentration of about 2 ppm or more, about 10 ppm or more, about 50 ppm or more, about 100 ppm or more, about 200 ppm or more, about 300 ppm or more, about 400 ppm or more, about 500 ppm or more, about 600 ppm or more, about 700 ppm or more, about 800 ppm or more, about 900 ppm or more, about 1000 ppm or more, about 11 ppm or more, about 1200 ppm or more, about 1300 ppm or more, about 1400 ppm or more, or about 1500 ppm or more.

9. The method of claim 8, where in the electrolyte solution has an Mg-equivalent concentration of about 1000 ppm or more.

10. The method of claim 1, wherein the one or more hydroxide solids comprises Mg(OH)<sub>2</sub>, Ca(OH)<sub>2</sub>, or both Mg(OH)<sub>2</sub> and Ca(OH)<sub>2</sub>.

11. The method of claim 1, wherein the one or more hydroxide solids comprises Mg(OH)<sub>2</sub>.

12. The method of claim 1, wherein the electroactive mesh cathode comprises a rotating disc cathode having the electroactive mesh disposed thereon.

13. The method of claim 1, further comprising removing the one or more hydroxide solids from the surface of the mesh.

14. The method of claim 13, wherein the removing the one or more hydroxide solids from the surface of the mesh comprises scraping the surface of the mesh or forcing a solution across the surface of the mesh using a high-pressure nozzle.

15. The method of claim 13, wherein removing the one or more hydroxide solids from the surface of the mesh comprises rotating the rotating disc cathode past a scraper, a metallic brush, or a blade.

16. The method of claim 1, wherein the electroactive mesh comprises a mesh cathode that comprises a metallic composition, non-metallic composition, or hybrid metallic and non-metallic composition.

17. The method of claim 16, wherein the mesh cathode comprises stainless steel, titanium oxide, carbon nanotubes, one or more polymers, graphite, or combinations thereof.

18. The method of claim 17, wherein the mesh cathode comprises stainless steel.

19. The method of claim 1, wherein the electroactive mesh comprises pores having a diameter in the range of about 0.1  $\mu$ m to about 10000  $\mu$ m.

20. The method of claim 1, further comprising forming alkalinized effluents having a pH greater than 9.

21. The method of claim 20, further comprising forming alkalinized effluents having a pH greater than 10.

22. The method of claim 1, wherein the anolyte comprises an acid.

23. The method of claim 22, wherein the anolyte has a pH of less than about 6.

24. The method of claim 1, further comprising providing a barrier to separate the catholyte and the anolyte.

25. The method of claim 24, wherein the barrier comprises a polymer.

26. The method of claim 25, wherein the barrier comprises cellulose, polyvinyl chloride, organic rubber, polyolefin, polyethylene, polypropylene, or any combination thereof.

27. The method of claim 1, wherein the alkaline material comprises a mafic material, ultramafic material, calcium-rich fly ash, or slag.

28. The method of claim 27, wherein the alkaline material comprises a mafic material or an ultramafic materials.

29. The method of claim 1, wherein electrolytically generating hydroxide ions is conducted at a current density of greater than 50  $\mu$ A/cm<sup>2</sup>.

30. The method of claim 1, wherein the one or more hydroxide solids comprise a hydroxide of a divalent metal ion.

\* \* \* \* \*